

1,096,636.

P. McILROY.  
COATED ARTICLE.  
APPLICATION FILED OCT. 16, 1913.

Patented May 12, 1914.

FIG. 2.



FIG. 1.



WITNESSES

J. Murrayfield  
W. C. Cooke

INVENTOR

Peter McIlroy,  
By J. W. Cooke,  
Attorney.

# UNITED STATES PATENT OFFICE.

PETER McILROY, OF PITTSBURGH, PENNSYLVANIA, ASSIGNOR TO ENAMELED METALS COMPANY, OF SHARPSBURG, PENNSYLVANIA, A CORPORATION OF PENNSYLVANIA.

## COATED ARTICLE.

1,096,636.

Specification of Letters Patent.

Patented May 12, 1914.

Application filed October 16, 1913. Serial No. 795,441.

To all whom it may concern:

Be it known that I, PETER McILROY, a citizen of the United States, and a resident of Pittsburgh, North Side, in the county of Allegheny and State of Pennsylvania, have invented a new and useful Improvement in Coated Articles; and I do hereby declare the following to be a full, clear, and exact description thereof.

10 My invention relates to coated articles and has special reference to the coating of metal articles, such as pipes, plates, etc.

In the manufacture of coated metal articles, such as what are known as galvanized pipes for electric conduit purposes, such conduits have been generally formed by a zinc coating electro-plated on the exterior of the pipe and an enamel or other coating on the interior. These articles such as conduits are 20 usually made of steel but may be made of cast iron or any ferrous metal. In the manufacture of these zinc-plated pipes there are two methods generally employed, one known as the continuous process in which the pipe 25 is electro-plated horizontally and the other in which the pipe is so treated perpendicularly. With the first named method it is possible to deposit the zinc without first applying what is known as a "strike" coat, as 30 the pipe can be brushed and cleaned and immediately plunged into the zinc bath so that it does not have time to tarnish. With the other or second named method it is impractical to zinc coat without first using a

35 "strike." The purpose of this "strike" is to deposit a coat of some metal which will adhere to the pipe more readily than zinc and up to the present time a copper "strike" has always been used and then the zinc coat-

40 ing is put on in the usual way in a separate tank. When no "strike" is used, it is a matter of chance whether the pipe will plate equally over its entire length, (as with this method, viz., perpendicularly, it is not practical to immerse the pipe in the zinc bath 45 soon enough after being cleaned to prevent slight oxidation taking place, and no article will plate equally over its entire surface unless the entire surface is equally clean).

50 When the "strike" is used the current employed in applying the "strike" acts as an electric cleaner, so that such pipe is cleaned equally throughout its entire length, and the "strike" coat is deposited uniformly all 55 over the pipe. The current, acting as an

electric cleaner, also forces out all acids and impurities that may be in the minute pores of the metal, allows the "strike" coat to be deposited in these pores and removes danger of "spotting out", which is liable to 60 occur on any plated article not properly cleaned.

The object of the present invention is to provide for using a "strike" coat in place of such copper strike, by which a better and 65 more uniform coating of zinc is deposited on the pipe than with the use of either the copper "strike" or with the process in which no "strike" is used, while the substituted "strike" for the copper "strike" is also 70 much cheaper than the latter.

To these ends my invention consists, generally stated, in the novel coated article, as hereinafter more specifically set forth and described and particularly pointed out in 75 the claims.

To enable others skilled in the art to which my invention appertains to construct and use my improved coated article, I will describe the same more fully, referring to 80 the accompanying drawing, in which:—

Figure 1 is a side elevation, partly broken away, of a pipe for electrical conduit purposes showing my invention applied thereto. Fig. 2 is a cross-section of the same. 85

Like symbols of reference herein indicate like parts in each of the figures of the drawing.

As illustrated in the drawing, 1 represents a pipe, which is formed of any suitable 90 metal, such as steel, and such pipe is subjected to the following treatment for using the same as a conduit for electric wires. The pipe is first immersed in an alkali bath to clean the same by removing all oils and 95 grease therefrom, after which it is pickled in an acid bath to further clean the same by removing the scale therefrom, and then it is immersed in a lime or other bath to neutralize the pickling acid. The pipe is then 100 brushed inside and outside in any suitable manner to remove any oxidation that may have taken place on the pipe after it has been exposed to the air from the last named bath, and after which it is again immersed 105 in an alkali cleaning bath to prepare it for the plating bath. The pipe is now ready to be electro-plated and this is accomplished in two operations or two coatings. In the first, a coating 2 is deposited on the pipe in 110

the usual electro-plating manner by immersing the pipe in a bath, and such coat is called a "strike" coat, which consists of a mixture of copper and zinc in certain proportions, as may be required, a preferred or good proportion being forty (40) per cent. of copper and sixty (60) per cent. of zinc, which practically makes a brass colored coating on the pipe. A coating of zinc is then applied on top of the combined copper and zinc alloy coating on the pipe by the usual electro-plating process in another separate bath. It will thus be seen that in my improved coated pipe, the "strike" coat applied thereto reduces all danger of what is known as "spotting out" to a minimum and the pipe finished with a much better color by being whiter and more uniform. The percentage of the pipe failing to plate properly with the zinc coating is greatly reduced, and practical experience has proven that about ninety-nine (99) per cent. of the output will plate perfectly, which is much higher than the first approved processes practised without a "strike" coat or with a copper "strike" coat. It has been practically proven that a pipe having a "strike" coat of the kind described, (before being plated with zinc, will never deteriorate through galvanic action taking place,) and it has also been proven that a pipe having a "strike" coat of either copper or the alloy described will show less corrosion than zinc alone, so that a "strike" coat of any kind is preferable to none at all.

Some of the advantages of a pipe coated as above described are as follows: It minimizes the danger of acid being left in the pores of the metal of the pipe to destroy the zinc coating. (Pipe coated in this manner has a better appearance, being whiter and more uniform in color.) The manu-

facturing cost is reduced owing to there being less imperfect coatings, while the copper "strike" coat is more expensive, as copper is sold at a higher price than zinc. The pipe as thus coated resists corrosion much better than pipe plated without a strike coat and it is possible to put a lighter coating of zinc on the pipe, if desired, than by the other known methods, and it also takes less time to put the described "strike" coat on than the copper "strike". With the zinc coating applied to the "strike" coating described, a more tenacious coating of the zinc will be had and a heavier coating of zinc can be applied without danger of peeling.

Various modifications and changes in the process described and in the proportions used, as well as in the application of the same may be resorted to without departing from the spirit of the invention or sacrificing any of its advantages.

What I claim as my invention and desire to secure by Letters Patent, is:—

1. A metal article having a strike coating of copper and zinc applied to the same and a coating of zinc applied to said first named coating.
2. A ferrous article having a strike coating of copper and zinc applied to the same and a coating of zinc applied to said first named coating.
3. A steel article having a strike coating of copper and zinc applied to the same and a coating of zinc applied to said first named coating.

In testimony whereof I, the said PETER MCILROY, have hereunto set my hand.

PETER MCILROY.

Witnesses:

S. E. HEDDEN,  
J. N. COOKE.